

1

2,831,761

**METHOD FOR PRODUCING LOW-CARBON FERROCHROMIUM**

Hugh S. Cooper, Cleveland, Ohio, assignor to  
Walter M. Weil, Cleveland, Ohio

No Drawing. Application May 10, 1956  
Serial No. 583,894

6 Claims. (Cl. 75—28)

This invention relates to the production of ferrochromium and particularly to the production of low-carbon ferrochromium by the decarburization of high-carbon ferrochromium. Though the invention is not limited to the production of ferrochromium having any particular ratio of chromium to iron, industrial uses of ferrochromium for most purposes require a percentage of chromium of at least 50% and generally at least 65%, a range of 65-75% being most commonly used as a master alloy in the production of stainless steel. Thus, the principal uses for the invention involve chromium contents of this order of magnitude.

In the production of many chromium-containing iron alloys, it is highly desirable to employ a ferrochromium master alloy having a low carbon content, generally of the order of 0.03% or less in the case of the production of stainless steel, unless the stainless steel also contains columbium or titanium to fix the carbon in the steel in such a manner that higher carbon contents can be tolerated without inter-granular corrosion.

For many years, ferrochromium of low carbon content has been prepared principally by a silicon reduction process in an open-arc electric furnace. This process is expensive to operate, and many efforts have been made to find a less expensive process for accomplishing the same end result.

More recently, it has been proposed to produce low-carbon ferrochromium by decarburizing high-carbon ferrochromium under subatmospheric pressure with a suitable oxidant for the carbon, the carbon being removed largely as carbon monoxide. Such a process is the subject of U. S. Patents 2,473,019 and 2,473,020 to Erasmus and U. S. Patent 2,473,021 to Spendelow et al. The inventions of these patents are presently being exploited commercially on a large scale using silica as the oxidant, a pelletized mixture of high-carbon ferrochromium and silica being heated under a relatively high vacuum and maintained at an elevated temperature sufficient to effect combination of the carbon with the oxygen of the silica. The silica also assists in removing excess sulfur, though it adds silicon to the alloy in the process. Thus, the resulting product is a low-carbon ferrochromium in pellet form having a relatively high silicon content. According to the above mentioned patents, the process is preferably conducted at a temperature above 1150° C. but below the temperature at which the reacting charge fuses. To obtain a practical rate of reaction while avoiding fusion, a temperature above the solidus temperature of the high-carbon ferrochromium, but below about 1300° C. (for 65% to 75% chromium content), is employed until the carbon content at the surfaces of the pellets approaches the eutectic composition, whereupon the temperature is reduced to below the eutectic temperature until the carbon concentration throughout the charge has dropped substantially below the eutectic percentage. Thereafter, the temperature may be raised and decarburization continued at as high a temperature as desired, provided only that the liquidus temperature of the ferro-

2

chromium is not reached before the decarburizing reaction is substantially complete.

According to U. S. Patent 2,473,021, the outer surfaces of the pellets of charge material are decarburized more rapidly than the interiors thereof, so that the outer surfaces approach the eutectic composition before substantial decarburization of the interiors of the pellets has occurred. Unless the temperature is reduced as the eutectic composition is approached in the outer surfaces of the pellets, these surfaces tend to fuse and form a skin which prevents further effective decarburization of the interiors of the pellets, so that continued heating converts the interiors of the pellets to a stone-like unreacted mass. To avoid this, it was proposed to reduce the temperature to below the eutectic temperature when the surfaces of the pellets approach the eutectic composition and to maintain the lower temperature until substantially the entire mass has passed through the eutectic composition. Thereafter, the temperature may be raised as decarburization proceeds without danger of fusion, provided the liquidus temperature is not too closely approached.

Decarburization of high-carbon ferrochromium according to this last described process is very slow, at best. According to the three patents referred to above, the process requires heating for upwards of 20 hours to reduce the carbon to the desired low concentration. In actual practice, when decarburizing many tons of alloy at a time, the heating cycle takes about one week. As noted above, decarburization is performed with the charge material in the form of compacted pellets, and these pellets retain their form during the process. Thus the final product is in the form of highly porous pellets, which have been found to be objectionable in many cases because of their tendency to float on top of a molten metal bath to which they are added, thus making it difficult to melt the product into the bath before it absorbs excessive amounts of nitrogen from the atmosphere, which gives undesirable properties to the resulting alloy.

The principal object of the present invention is to accelerate the process of decarburizing high-carbon ferrochromium by heating with an oxidant so as to improve the economy of the process.

A further object of the invention is to accomplish the foregoing objective, while still removing excess sulfur from the charge material, without increasing the silicon content of the product.

Still another object of the invention is to provide a process for decarburizing high-carbon ferrochromium by heating with an oxidant without the necessity for compressing and bonding a mixture of the reactants into cemented pellets.

In accordance with the present invention, the rapidity and, therefore, the economy of the decarburizing reaction are greatly enhanced and, if desired, the low-carbon ferrochromium product may readily be produced in the form of non-porous, massive metal more suitable for many metallurgical uses. Moreover, in accordance with the present invention, the high sulfur content of the high-carbon starting material may be reduced to a satisfactory value without producing the high silicon content which results from the use of silica as the oxidant.

The present invention is based on the discovery that it is possible to use iron oxide, chromium oxide, or a mixture thereof as the oxidant, while carrying out the decarburizing reaction at a higher and substantially uniform temperature through the eutectic stage, thus greatly accelerating the reaction to the point where it may be completed in a period of from one to two hours. It has been discovered that, at such higher reaction temperatures, sulfur in the charge material is substantially reduced without the use of silica as an oxidant, and that the decarburizing

reaction may be carried out at such higher temperatures without fusion of the reactants and consequent retardation of the reaction, which has heretofore been considered inevitable if the charge passes through the eutectic composition above the eutectic temperature.

In accordance with the invention, finely comminuted high-carbon ferrochromium is mixed with the metal oxide, also in a finely comminuted form. For convenience in handling, this dry mixture may simply be pressed into lumps or cakes of any convenient size without employing any bonding agent.

The mixture of high-carbon ferrochromium and metal oxide, either in loose comminuted form or lump or brick form, with or without a bonding agent, is first heated to a temperature in the range of about 800° to 1000° C. in a suitable reaction chamber, while reducing the pressure in the chamber until a high vacuum is obtained, preferably less than 0.1 mm. of mercury absolute pressure. The temperature in this range is maintained long enough for the entire charge to have reached such temperature and for air and gas entrained in the reaction mass to be effectively reduced to a negligible quantity. Thereupon the temperature of the mass is preferably raised as quickly as the charge will absorb the heat, to a point well above the solidus temperature of the ferrochromium, e. g., about 1325°-1425° C., while maintaining the low subatmospheric pressure to the extent that it is practical to do so during the rapid evolution of carbon monoxide resulting from the decarburizing reaction. Under these conditions, the carbon content of the ferrochromium is rapidly reduced to below the eutectic composition with no objectionable tendency of any part of the charge to fuse.

When the carbon content has been reduced to well below the eutectic composition, the temperature may be further raised gradually to about 1500° C. or so until decarburization and evolution of carbon monoxide have ceased, as evidenced by the ability to maintain a substantially stable vacuum in the reaction chamber. Thereupon, if desired, the temperature may be further raised to above the melting temperature to convert the decarburized ferrochromium to a molten condition suitable for pouring from the reaction chamber into molds. Preferably, before raising the temperature above about 1500° C. for this purpose, an inert gas is bled into the reaction chamber so that the gas pressure will inhibit vaporization of chromium during the melting operation. However, the tendency for such vaporization to occur to any appreciable extent is slight because of the fact that the chromium is present as an alloy with iron and is less rapidly vaporized in this condition.

When the charge material has been preliminarily compacted or formed into cemented pellets, the decarburizing reaction leaves the product in substantially the same pelletized or lump condition, except that it is porous due to the rapid evolution of gas from the mass during the decarburizing reaction. The above melting step converts the product into dense massive metal.

Instead of finally raising the temperature in the reaction chamber above the melting point of the decarburized ferrochromium, the temperature may be raised only sufficiently to sinter or partially fuse the material into a coherent mass. Such mass may be broken up and the fragments readily cold pressed into coherent, dense masses of a size and shape suitable for use as an alloying ingredient in the manufacture of steel.

Despite the fact that the charge material, when handled in accordance with the present invention, apparently passes through the eutectic composition at a temperature at which it should theoretically be in a molten condition, it appears that no melting occurs during the process. When the charge has been uniformly heated to well above the solidus temperature before the decarburizing reaction is initiated, it appears that the reaction proceeds at such a rate throughout the mass that the eutectic com-

position does not exist for a long enough time for any appreciable fusion to occur. Thus, higher reaction temperatures than have heretofore been used may be employed without difficulty and may be maintained continuously above the eutectic temperature from the time the reaction is initiated until the carbon content has been reduced to well below the eutectic composition. After passing through the eutectic composition, the liquidus curve rises sharply with further reductions in carbon content. Below about 1% carbon, the temperature may be gradually raised to a considerably higher level as the carbon content is further reduced, preferably while avoiding temperatures above the liquidus curve until decarburization is complete.

To illustrate the operation of the invention, three examples are given below of runs made on a high-carbon ferrochromium of the following analysis:

|                      | Percent by weight |
|----------------------|-------------------|
| Chromium             | 68.06             |
| Carbon               | 4.59              |
| Silicon              | 1.70              |
| Sulfur               | 0.055             |
| Iron (by difference) | 25.595            |

In each example, the high-carbon ferrochromium to be decarburized and the oxidant or oxidants were comminuted so that substantially all would pass through a 100-mesh screen. These finely divided reactants were thoroughly mixed and formed into briquettes by simply pressing them in a dry state into a mold with no added binder. The reactants were heated in each example in a zirconia crucible contained in a molybdenum resistor-type vacuum furnace. The degree of vacuum was measured at various stages in the process with a McLeod gauge in mm. of mercury absolute pressure.

#### Example I

Iron oxide as an oxidant was mixed with the high-carbon ferrochromium in the ratio of 26.25 parts to 100 parts by weight. The briquetted mixture was placed in the furnace, and the furnace was evacuated to about .002-.003 mm. pressure. The furnace temperature was then raised to about 850° C. and held for about 30 minutes to degas the charge and heat it uniformly throughout its mass. Because of the release of occluded gases, the pressure in the furnace rose to about .150 mm. during this preheating operation, the rise in pressure being so slight as to indicate that decarburizing had not yet commenced.

The temperature was then quickly raised to about 1375° C., whereupon rapid evolution of carbon monoxide occurred. This further impaired the degree of vacuum that could be maintained in the furnace to such an extent that no vacuum readings could be made on the McLeod gauge. After about 2 hours of heating at this temperature, while continuing to pump out the evolved gas, a steady pressure reading of about .003 mm. on the McLeod gauge was again obtained, indicating that decarburization had virtually ceased. The temperature was then quickly raised to 1650° C. to melt the charge, while maintaining the vacuum. Finally, the furnace was allowed to cool, and the charge was removed and analyzed. The analysis of the product was as follows:

|          | Percent by weight |
|----------|-------------------|
| Chromium | 54.86             |
| Carbon   | 0.033             |
| Sulfur   | 0.022             |

The balance of the product, of course, was made up of the iron and silicon in the original ferrochromium charge and in the iron oxide mixed therewith.

#### Example II

Chromium oxide as an oxidant was mixed with the high-carbon ferrochromium in the ratio of 20 parts to

100 parts, by weight, and the briquetted mixture was placed in the furnace and subjected to the same operations described in Example I, except that the heating to degas the charge was continued for about 1 hour, the decarburizing temperature was between 1350° and 1375° C. and was maintained for only about 1½ hours, and the final melting temperature employed was about 1675° C. Analysis of the final product showed the following composition:

|          | Percent by weight |
|----------|-------------------|
| Chromium | 73.14             |
| Carbon   | 0.020             |
| Sulfur   | 0.015             |

*Example III*

A combination of 5 parts of chromium oxide and 7½ parts of iron oxide was mixed with 100 parts of the high-carbon ferrochromium, by weight, and the mixture was subjected to the same operations described in Example I, except that the preliminary heating was conducted by slowly raising the temperature of the entire mass to about 900° C. over a period of about ½ hour. The temperature was then raised rapidly to about 1300° C., and a decarburizing temperature was maintained between 1310° and 1375° C. for about 2 hours. The final melting temperature was about 1585° C. The analysis of the product was as follows:

|          | Percent by weight |
|----------|-------------------|
| Chromium | 62.52             |
| Carbon   | 0.022             |
| Sulfur   | 0.023             |

From the foregoing examples, it will be observed that iron oxide, chromium oxide, and mixtures thereof are substantially equally effective in decarburizing ferrochromium and in reducing the sulfur content. The choice between the three types of oxidant is governed largely by the desired final chromium-to-iron ratio, which is increased or decreased to the extent that chromium may be present in a greater or lesser ratio in the oxide or mixture of oxides used as the oxidant.

Though, in all three instances, the charge was maintained well above the eutectic temperature of approximately 1275° C. throughout the decarburizing operation, observation of the charge as the carbon content passed through the eutectic composition showed no visible sign of fusion, and the briquettes retained their original form until the final melting step. The great rapidity of the decarburizing operation demonstrated that the formation and escape of carbon monoxide was at least not significantly hindered by fusion of the charge, if any fusion at all occurred.

As noted above, a possible explanation for the rapidity of the decarburizing reaction and for the apparent lack of fusion at temperatures at which the charge would have been expected to melt, while at or near the eutectic composition, is that the composition of the charge changed so rapidly at the high decarburizing temperatures employed that insufficient time for fusion was available. It is believed that preheating the charge uniformly to a temperature below but close to that at which decarburization commences, for degassing the charge, contributes to the surprising results obtained by making rapid and uniform heating of the entire charge to a temperature above 1300° C. easier to achieve. Whatever the explanation may be, however, the efficiency of the decarburizing operation and the lack of any sign of fusion until the final melting temperature is produced are contrary to what would be expected from the prior art.

In addition, contrary to the teachings of the prior art, it is unnecessary for the oxidant to contain any silica in order to reduce the sulfur content when operating at the higher temperatures employed in accordance with the present invention. Thus, sulfur may be reduced without increasing the silicon content of the ferrochromium. In

general, chromium oxide is preferred for this purpose, as well as being desirable for increasing the chromium content of the final product.

From the foregoing disclosure of the invention, it will be apparent that the various objectives of the invention have been achieved in a simple and practical manner, producing a superior product in a small fraction of the time heretofore required in any previously known, simple decarburizing operation.

While the invention has been illustrated with reference to specific examples, it is to be understood that the invention is not limited to the particular conditions disclosed in the examples and that numerous variations thereof may be employed within the scope of the appended claims.

What is claimed is:

1. The method of decarburizing ferrochromium containing in excess of 3% carbon by weight, comprising mixing said ferrochromium and an oxidant, both in comminuted form, the oxidant being selected from the class consisting of iron oxide, chromium oxide, and mixtures thereof and being present at least in the amount required to supply oxygen sufficient to combine as CO with the carbon to be eliminated from said ferrochromium, heating said mixture uniformly and under subatmospheric pressure to a temperature between about 800° and 1000° C. to degas the same, quickly raising the temperature of said mixture to an initial reaction temperature in the range above the eutectic temperature but below the liquidus temperature of said ferrochromium while maintaining said subatmospheric pressure, and maintaining said subatmospheric pressure and a reaction temperature above said eutectic temperature until the carbon remaining in said ferrochromium is below 1% by weight.

2. The method of decarburizing ferrochromium containing from about 65% to 75% chromium and in excess of 3% carbon by weight, comprising mixing said ferrochromium and an oxidant, both in comminuted form, the oxidant being selected from the class consisting of iron oxide, chromium oxide, and mixtures thereof and being present at least in the amount required to supply oxygen sufficient to combine as CO with the carbon to be eliminated from said ferrochromium, heating said mixture uniformly and under subatmospheric pressure to a substantially non-decarburizing temperature above 800° C. to degas the same, quickly raising the temperature of said mixture to an initial reaction temperature in the range between 1300° and 1425° C. but below the liquidus temperature of said ferrochromium while maintaining said subatmospheric pressure, maintaining said subatmospheric pressure and a reaction temperature in said range until the carbon remaining in said ferrochromium is below 1% by weight, and finally raising the temperature of the ferrochromium above its melting point to coalesce the same into a non-porous mass.

3. The method of decarburizing ferrochromium containing in excess of 3% carbon by weight, comprising mixing said ferrochromium and an oxidant, both in comminuted form, the oxidant being selected from the class consisting of iron oxide, chromium oxide, and mixtures thereof and being present at least in the amount required to supply oxygen sufficient to combine as CO with the carbon to be eliminated from said ferrochromium, heating said mixture uniformly and under subatmospheric pressure to a temperature between about 800° and 1000° C. to degas the same, quickly raising the temperature of said mixture to an initial, non-fusing, reaction temperature above the eutectic temperature of said ferrochromium while maintaining said subatmospheric pressure, maintaining said subatmospheric pressure and a reaction temperature above the eutectic temperature until the carbon remaining in said ferrochromium is below 1% by weight, surrounding the decarburized ferrochromium with an atmosphere of an inert gas, and finally raising the tempera-

60  
65  
70  
75

ture of the ferrochromium above its melting point to coalesce the same into a non-porous mass.

ture of the decarburized ferrochromium above its melting point to coalesce the same into a non-porous mass.

4. The method of decarburizing ferrochromium containing in excess of 3% carbon by weight, comprising mixing said ferrochromium and an oxidant, both in comminuted form, the oxidant being selected from the class consisting of iron oxide, chromium oxide, and mixtures thereof and being present at least in the amount required to supply oxygen sufficient to combine as CO with the carbon to be eliminated from said ferrochromium, heating said mixture uniformly and under subatmospheric pressure to a substantially non-decarburizing temperature above 800° C. to degas the same, quickly raising the temperature of said mixture to an initial reaction temperature in a range above the eutectic temperature of said ferrochromium but below 1425° C. while maintaining said subatmospheric pressure, and maintaining said subatmospheric pressure and a reaction temperature in said range until the carbon remaining in said ferrochromium is below 1% by weight.

5. The method of decarburizing ferrochromium containing in excess of 3% carbon by weight, comprising mixing said ferrochromium and an oxidant, both in comminuted form, the oxidant being selected from the class consisting of iron oxide, chromium oxide, and mixtures thereof and being present at least in the amount required to supply oxygen sufficient to combine as CO with the carbon to be eliminated from said ferrochromium, heating said mixture uniformly and under subatmospheric pressure to a substantially non-decarburizing temperature above 800° C. to degas the same, quickly raising the temperature of said mixture to an initial reaction temperature in a range above the eutectic temperature of said ferrochromium but below 1425° C. while maintaining said subatmospheric pressure, maintaining said subatmospheric pressure and a reaction temperature in said range until

the carbon remaining in said ferrochromium is below 1% by weight, surrounding the decarburized ferrochromium with an atmosphere of an inert gas, and finally raising the temperature of the decarburized ferrochromium above its melting point to coalesce the same into a non-porous mass.

6. The method of decarburizing ferrochromium containing from about 65% to 75% chromium and in excess of 3% carbon by weight, comprising mixing said ferrochromium and an oxidant, both in comminuted form, the oxidant being selected from the class consisting of iron oxide, chromium oxide, and mixtures thereof and being present at least in the amount required to supply oxygen sufficient to combine as CO with the carbon to be eliminated from said ferrochromium, heating said mixture uniformly and under subatmospheric pressure to a temperature between about 800° and 1000° C. to degas the same, quickly raising the temperature of said mixture to a reaction temperature in the range between 1300° and 1425° C. below the liquidus temperature of said ferrochromium, maintaining said subatmospheric pressure and a reaction temperature in said range until the carbon remaining in said ferrochromium is below 1% by weight, surrounding the decarburized ferrochromium with an atmosphere of an inert gas, and finally raising the temperature of the decarburized ferrochromium above its melting point to coalesce the same into a non-porous mass.

References Cited in the file of this patent

UNITED STATES PATENTS

|            |                  |                |
|------------|------------------|----------------|
| Re. 21,500 | Rennerfelt       | July 2, 1940   |
| 2,432,856  | Brace            | Dec. 16, 1947  |
| 2,473,021  | Spendelow et al. | June 14, 1949  |
| 2,763,918  | Megill           | Sept. 25, 1956 |
| 2,776,882  | Chadwick         | Jan. 8, 1957   |